

## UNITED STATES PATENT OFFICE

LEVIS MILLER BOOTH, OF PLAINFIELD, NEW JERSEY

## PROCESS OF MANUFACTURE OF PULP AND PAPER

No Drawing.

Application filed October 22, 1927. Serial No. 228,104.

This invention relates to the process of manufacturing pulp and paper by treating pulp which has been digested by an alkaline process with a coagulating salt and reducing 5 or dispensing with the usual washing process and adding chlorine.

In the process of manufacturing paper or board, as for example kraft or straw paper or board, the wood chips or straw have here- 10 tofore been treated by an alkaline process for the purpose of loosening the lignins, resins and other non-fibrous substances from the fibrous materials. The former were then separated from the latter by a washing proc- 15 ess which results in the production of voluminous quantities of alkaline wash water carrying non-fibrous organic matter, as well as small amounts of fibrous material. By processes heretofore practiced the alkaline 20 wash water, together with its burdens of mineral and organic matter is either wasted or treated by recovery or disposal processes.

I have found that it is possible to increase the yield of paper or board and at the same 25 time to materially lessen the volume of wash water required by terminating the pulp washing process at a time when appreciable amounts of alkali still persist, which if left free in the pulp are detrimental in the sub- 30 sequent paper or board making processes and to the product. I may eliminate washing entirely.

After digesting the pulp by an alkaline process I introduce into the pulp washer or 35 washer beater or subsequently, an acid salt having a coagulating effect which permits the use of pulp containing more of alkali and non- 40 fibrous matter than it has been feasible to employ in the manufacture of paper or board of the kind and quality commonly acceptable in commerce. One example of the application of my process which I have found to be practicable is as follows:

For the manufacture of straw paper or 45 board straw is cooked in the presence of lime. The pulp is then washed for the purpose of removing the excess lime and non-fibrous material. In one instance the washing process has heretofore been continued for a period 50 of approximately three hours to produce a

suitable quality of pulp. In my improved process I discontinue the washing after a fraction of the usual washing period or do not wash at all and add a coagulating substance, such as sulphate of aluminum, ferrous 55 sulphate, or ferric sulphate and ferric chloride with the addition of chlorine. The treatment which I effect causes the neutralization of the alkali to the required extent and further insures the retention of non- 60 fibrous and fibrous material in the finished product which by processes heretofore used would be wasted or have to be recovered by a separate process.

Besides conserving raw material I ma- 65 terially reduce the volume of wash water required or eliminate it entirely.

## Claims.

1. The process of treating partially washed or unwashed pulp which has been digested 70 by an alkaline process which consists of adding to such pulp a coagulating metallic salt and chlorine.

2. The process of treating partially washed or unwashed pulp which has been digested by 75 an alkaline process which consists of adding to such pulp ferrous sulphate and chlorine.

3. The process of treating partially washed or unwashed pulp which has been digested by an alkaline process which consists of 80 adding to such pulp ferric sulphate, ferric chloride and chlorine.

4. The process of treating partially washed or unwashed pulp which has been digested by an alkaline process which consists of 85 adding an acidifying substance and chlorine.

LEVIS MILLER BOOTH.

90

95

100